

March 28, 1933.

A. R. GOODHUE

1,902,815

## MANUFACTURE OF STEEL SHEETS

Filed Nov. 21, 1931



*Inventor:*  
ARCHIE R. GOODHUE,  
*by:* *Usina & Rauber*  
*his Attorneys.*

## UNITED STATES PATENT OFFICE

ARCHIE R. GOODHUE, OF VANDERGRIFT, PENNSYLVANIA, ASSIGNOR TO AMERICAN SHEET AND TIN PLATE COMPANY, A CORPORATION OF NEW JERSEY

## MANUFACTURE OF STEEL SHEETS

Application filed November 21, 1931. Serial No. 576,596.

This invention relates to the manufacture of high silicon electrical steel sheets, and has for its object the provision of a novel method of manufacturing such sheets whereby they are cleaned of all scale and have a smooth, clean surface, so as to provide an improved space factor over such sheets as heretofore manufactured.

High silicon electrical steel sheets are used mainly in the construction of those parts of electrical apparatus, such as the cores of transformers, generators and the poles of motors and dynamos, that demand a high magnetic permeability and electrical resistance of greatest efficiency. In the construction of these apparatus the high silicon electrical steel sheets are stacked one upon the other, with light insulation between the sheets, and it is important, in order to get the greatest efficiency from the apparatus, that the sheets should stack tightly against a separate insulation so as to eliminate the air pockets in the structure. This tight or close stacking of the sheets is known as "the space factor" and it is important, in order to have the best possible space factor, that the surfaces of the sheets be smooth and clean, so as to eliminate any unnecessary spacing or air pockets between the sheets.

Briefly, this method consists in an improved series of pickling and cleaning steps after the sheets have been annealed, which steps serve to completely remove all scale and foreign matter from the surfaces of the sheets.

The drawing forming part of this specification illustrates diagrammatically the apparatus used in carrying out the several steps of this invention.

The high silicon steel sheets to be treated in accordance with this invention are generally first normalized, cold rolled and box annealed, although any of the usual steps of manufacture may be used up to the annealing step. After the sheets are annealed they are mounted in a suitable pickling rack 1 in spaced relation to each other. The spaced relation of the sheets may be maintained in any manner, such as by the use of separating pins, commonly used for this purpose. After

the sheets are mounted in the pickling rack they are immersed in a pickling solution of approximately 7½ per cent. sulfuric acid, which is maintained at from 170 to 180 degrees Fahrenheit, contained in a pickling tank 2 for a period of from four to twelve minutes.

The pickling solution in the tank 2 is discarded when the Baumé exceeds 20 degrees. No inhibitor is used in the above picking solution.

After the sheets have been suitably pickled in the solution in the tank 2 the rack of sheets will be removed from the tank 2 and immersed in a clean, cold water bath in a tank 3, where they may be agitated or otherwise manipulated to thoroughly wash the sheets so as to remove all loose scale and to cool the sheets down to room temperature. The cooling of the sheets at this point in the process is essential, since the hot sheets should not be immersed in the next solution.

After the sheets have been thoroughly cleaned and cooled the rack 1 will be removed from tank 2 and lowered into the tank 4, which contains a ¾ to 2 per cent. nitric acid solution maintained at approximately 70 degrees Fahrenheit. The sheets are allowed to remain in the nitric acid solution in the tank 4 for from two to five minutes. This solution serves to soften and loosen substantially all the oxid and scale remaining on the surfaces of the plates. It is important that the nitric acid solution in the tank 4 be maintained in a substantially fresh condition, and the solution, therefore, is discarded after every five or six batches of plates have been immersed therein.

The rack of sheets is removed from the tank 4 and is next lowered into the tank 5 containing clean, cold water, where it is suitably manipulated to thoroughly wash the sheets and remove all the oxid, scale and other foreign matter loosened or softened by the nitric acid. The rack of sheets is removed from the tank 5 and lowered into the tank 6 containing an alkaline solution such as a solution of soda ash in water, which solution serves to neutralize any acid still re-

90

95

100

maining on the plates, so as to prevent further reaction with the metal.

The rack of sheets is next removed from the tank 6 and the cleaned sheets are removed from the rack 1 and piled upon a table 7, where they are then fed singly through the remaining apparatus for the remaining successive steps of the method. The sheets are singly fed from the table 7 continuously through a bosh 8 containing approximately a 7 per cent. solution of sulfuric acid maintained at approximately 200 degrees Fahrenheit. The sheets pass from the bosh 8 through a pair of wringer rollers 9 which squeeze the major portion of the water from their surfaces and then pass continuously through suitable pinch-rolls 10 and between top and bottom water sprays 11 which provide a continuous forced spray of clean, hot water against both top and bottom surfaces of the sheets to thoroughly wash the sheets and remove all acid from their surfaces.

The sheets pass from the water sprays 11 through wringer rollers 12 which squeeze the major portion of the water from their surfaces and serve to feed the sheets forwardly between a pair of upper and lower air blast nozzles 13 which provide a continuous forced blast of hot air against the sheets to dry all water from their surfaces. The sheets pass forwardly from the air nozzles 13 through a heated oven 14 in which they are baked or heated sufficiently to remove all entrapped moisture from the sheets and provide a finished product which has a scale-free and clean surface.

The 7 per cent. sulfuric acid solution in the bosh 8 is preferably discarded and a new solution supplied to the bosh after approximately 30,000 to 40,000 pounds of sheets have been treated or have passed through the bosh 8.

While I have described certain specific apparatus for carrying out this novel method, it will be understood that I do not wish to be limited thereto, since various forms of apparatus may be used for carrying out my method, and the steps of the method may be varied within the scope of the appended claims without departing from the scope of my invention.

I claim:

1. The method of producing scale-free, clean, high silicon electrical steel sheets, which consists in spacing the sheets, after being annealed, maintaining a batch of said sheets in spaced relation, pickling said sheets in a hot sulfuric acid solution, washing said pickled sheets in clean water to remove loose scale, pickling said washed sheets in a nitric acid solution, washing said sheets after said last named pickling step in clean water, then immersing said sheets in an alkaline bath, passing said sheets through a sulfuric acid

solution, washing said sheets to remove all traces of acid and then drying said sheets.

2. The method of producing scale free, clean, high silicon electrical steel sheets which consists in spacing the sheets, after being annealed, maintaining a batch of said sheets in spaced relation, pickling said sheets in a hot sulfuric acid solution, washing said pickled sheets in clean, cold water to remove loose scale and cool said sheets to approximately room temperature, pickling said washed sheets in a nitric acid solution, washing said sheets after said last named pickling step in clean, cold water, then immersing said sheets in an alkaline bath, passing said sheets singly through a sulfuric acid solution heated to approximately the boiling point, washing said sheets to remove all traces of acid, and then drying said sheets by applying heat.

3. The method of producing scale-free, clean, high silicon electrical steel sheets which consists in spacing said sheets, after being annealed, maintaining a batch of said sheets in spaced relation, pickling said batch of sheets, washing said pickled sheets to remove loose scale, cooling said sheets to approximately room temperature, pickling said washed and cooled sheets in a nitric acid solution having a temperature of not over 70 degrees Fahrenheit, washing said sheets after said last named pickling step in clean, cold water, then immersing said sheets in an alkaline bath, immersing said sheets in a sulfuric acid solution and removing the acid from said sheets and drying said sheets by applying heat.

4. The method of producing scale-free, clean, high silicon electrical steel sheets which consists in spacing said sheets, after being annealed, maintaining a batch of said sheets in spaced relation, pickling said batch of sheets for from four to twelve minutes in a 7½ per cent. sulfuric acid solution at from 170 to 180 degrees Fahrenheit and below 20 degrees Baumé, without an inhibitor, washing said batch of pickled sheets in clean, cold water to remove loose scale and to cool said sheets to approximately room temperature, pickling said batch of washed sheets in a ¾ to 2 per cent. nitric acid pickling solution maintained at approximately 70 degrees Fahrenheit for from two to five minutes, washing said batch of sheets after said last named pickling step in clean, cold water, then immersing said sheets in an alkaline bath, passing said sheets singly through an approximately 7½ per cent. sulfuric acid solution heated to approximately the boiling point, washing said sheets with hot water to remove the acid, and then drying said sheets by applying heat thereto.

5. The method of producing scale-free, clean, high silicon electrical steel sheets which consists in spacing said sheets, after being annealed, maintaining a batch of said

sheets in spaced relation, pickling said batch of sheets for from four to twelve minutes in a hot sulfuric acid solution, washing said batch of pickled sheets in clean, cold water  
5 to remove the loose scale and to cool the batch of sheets to approximately room temperature, pickling said batch of washed sheets for from two to five minutes in a  $\frac{3}{4}$  to 2 per cent. nitric acid pickling solution, washing said batch of sheets after said last named pickling step in clean, cold water, then immersing said batch of sheets in an alkaline bath, separating said batch of sheets and passing said sheets singly through a hot sulfuric acid solution, removing the acid and washing said sheets with hot water, and then drying said sheets.

In testimony whereof, I have hereunto set my hand.

20

ARCHIE R. GOODHUE.

25

30

35

40

45

50

55

60

65